

# UNITED STATES PATENT OFFICE.

ALBERT L. CLAPP, OF BRAINTEE, MASSACHUSETTS, ASSIGNOR TO REGINALD W. BIRD,  
OF FRAMINGHAM, MASSACHUSETTS.

## FIBROUS MATERIAL AND METHOD OF MAKING THE SAME.

1,269,905.

Specification of Letters Patent. Patented June 18, 1918.

No Drawing.

Application filed July 29, 1915. Serial No. 42,592.

To all whom it may concern:

Be it known that I, ALBERT L. CLAPP, a citizen of the United States, and a resident of Braintree, in the county of Norfolk and State of Massachusetts, have invented certain new and useful Improvements in Fibrous Materials and Methods of Making the Same, of which the following is a specification.

10 The object of the present invention, broadly stated, is two-fold: first, to produce a soft porous absorbent felt-like material, and, second, to utilize waste or scrap leather, which otherwise would be burned or unused commercially. A further object 15 of the invention is to produce a felt-like sheet material which can be used as the base or foundation in the manufacture of wall board, flooring, prepared roofing and the like.

According to my invention I subject scrap leather to the action of a beating engine, with sufficient water added, to disintegrate it into a fibrous pulpy mass. Scrap 25 leather of any kind may serve as the initial stock to be treated. The treatment of disintegration is continued until the fibrous mass is in condition to be run in a web onto a Fourdrinier or other equivalent form of 30 paper-making machine.

After being reduced to a soft pulpy fibrous mass, I add to the stock a small quantity of potassium or sodium bichromate, and a small quantity of calcium hydroxid, 35 sodium carbonate or the like, partially to neutralize the tannic acid in the leather, and to soften the fibers and render them absorbent when dry. The mixture is thoroughly beaten in the beating engine, and 40 then by any suitable machine or apparatus is formed into sheets of the desirable thickness, and then run through drying rolls, much in the same manner that cellulose fiber or wood pulp is formed into sheets of 45 paper.

Preferably, I add to the raw stock a quantity of cellulose fiber, such as mixed waste paper, rags, wood pulp or the like.

As an example of the method of carrying out my process, I may recite the following:

I load a beating engine with 1,000 pounds of leather scrap, and 200 pounds of waste

paper. Sufficient water is added to allow the stock to circulate in the beater. The 55 beater is then started in operation and the beating action is continued until the stock is gradually beaten out or disintegrated into a homogeneous pulpy fibrous state. The addition of the waste paper or its 60 equivalent prevents the leather fibers from sinking or settling in the aqueous mixture. When the pulpy mass has reached a condition when it may be run into a "wet machine" or into a Fourdrinier or other web-forming machine, I add to the mixture 5% to 10% by weight of bichromate of 65 potash or soda, and about 2% of sodium carbonate. After being thoroughly mixed in the beater, the mass is then formed into 70 sheets, either of predetermined or indeterminate lengths, and dried.

Such sheets are relatively soft, porous or absorbent, very much like wool felt. In 75 this condition they are saturated or impregnated with suitable compounds, such as waxes, oils, pitches, asphalts, resins or the like, according to the particular use to which they are to be put. For example, when they are to be employed in the manufacture of prepared roofings, they may be saturated with asphalt or other equivalent hydrocarbon compounds, and then coated with a relatively high-melting-point pitch or asphalt.

If desired, during the treatment of the raw stock, it may be heated to a temperature of say, not over 110° F., immediately prior to the addition of the bichromate and the carbonate of soda. Instead of adding 90 these ingredients at the same time, I sometimes first beat in the lime, or the carbonate of soda, before adding the bichromate.

Having thus described my product, and a method of making the same, what I claim is:

1. The herein described process of making felt for roofing which consists in disintegrating scrap leather into a fine fibrous pulpy mass, adding a softening agent and 100 then forming the mass into soft porous sheets of the desired thickness.

2. The herein described process of making felt for roofing which consists in disintegrating scrap leather and cellulose fiber 105 into a fibrous pulpy mass of the consistency

of paper stock, adding a softening agent and then forming the mass into soft porous sheets.

3. The herein described process of making felt for roofing which consists in disintegrating scrap leather into a fibrous pulpy mass, adding bichromate of soda or potash and carbonate of soda or its equivalent, mixing the same thoroughly in the pulpy mass, and then forming the mass into soft porous sheets.

4. The herein described process of making felt for roofing which consists in disintegrating scrap leather into a fibrous mass, forming the same into pulp with an admixture of cellulose, adding bichromate of soda or potash to the pulp, and then forming the pulp into soft porous absorbent sheets.

20 5. A felt-like sheet consisting essentially

of thoroughly disintegrated leather fiber and a softening agent, and which is soft, porous and absorbent.

6. A felt-like sheet consisting principally of thoroughly disintegrated leather fiber, a softening agent, and intermingled cellulose, such sheet being soft, porous, and absorbent.

7. A felt of which the base is disintegrated leather fiber, and having characteristics of porosity and absorption similar to those of a woolen or rag felt.

8. A soft, spongy, springy material composed in large measure of disintegrated leather fibers having united therewith the product of reaction between sodium or potassium bichromate and tannic acid.

In testimony whereof I have affixed my signature.

ALBERT L. CLAPP.